# EUROPEAN PATENT SPECIFICATION

(11) **EP 3 754 000 B1**
(45) Date of publication and mention of the grant of the patent: **01.01.2025**
(21) Application number: 19754985.0
(22) Date of filing: 15.02.2019
(51) Int. Cl.: C10M 111/04, C10M 101/02, C10M 105/38, C10M 107/34, C10M 137/04, C10N 30/00, C10N 30/04, C10N 30/10, C10N 40/06, C10N 40/08, C10N 40/12, C10N 40/30, C10M 169/04, C10N 30/02, C10N 20/02, C10N 30/06

(54) **LUBRICATING OIL COMPOSITION**
SCHMIERÖLZUSAMMENSETZUNG
COMPOSITION D'HUILE LUBRIFIANTE

(30) Priority: 16.02.2018 JP 2018026369
(43) Date of publication of application: 23.12.2020
(73) Proprietor: IDEMITSU KOSAN CO., LTD., Tokyo 100-8321 (JP)
(72) Inventor: SEKIGUCHI, Hiroki, Ichihara-shi, Chiba 299-0107 (JP)
(74) Representative: Hoffmann Eitle
(86) International application number: PCT/JP2019/005711
(87) International publication number: WO 2019/160123

(56) References cited:
- EP-A1- 0 524 783
- JP-A- 2011 516 637
- JP-A- 2013 023 596
- JP-A- 2015 004 028
- JP-A- 2018 009 106

## Description

### Technical Field

The present invention relates to a lubricating oil composition used in turbomachinery, compressors, hydraulic equipments, or machine tools, and a method of using the lubricating oil composition.

### Background Art

A lubricating oil composition for use in instruments including various turbomachinery such as steam turbines and gas turbines, compressors such as rotary gas compressors and reciprocating compressors, hydraulic equipments, and hydraulic units of machine tools is used while circulating in a high-temperature environment system for a long period of time.

When the lubricating oil composition is used for a long time under high temperature environments, it is susceptible to sludge precipitation according to oxidative deterioration. The precipitated sludge adheres to, for example, a bearing of a rotor to generate heat, thereby providing a risk of bearing damage, or may clog a filter arranged in a circulation line, or may deposit on a control valve, thereby often causing control system operation failures, etc.

Therefore, improvement in the effect of preventing sludge precipitation is required for the lubricating oil composition which is used while circulating in a high-temperature environment system for a long period of time.

For example, PTL 1 discloses a lubricating oil composition for air compressors, the composition including a synthetic base oil which is a mixed oil of a polyglycol-based synthetic oil and an ester-based synthetic oil, and one or more amine-based antioxidants selected from a specific compound group such as asymmetric diphenylamine-based compounds.

According to PTL 1, the lubricating oil composition for air compressors shows a result of preventing sludge precipitation while appropriately preventing oxidation.
EP 0 524 783 A1 describes lubricating oil compositions comprising a polyether with an alkyl or alkylphenyl group having 7 to 30 carbon atoms at one end of the molecule, and the other end of the molecule is a hydroxyl group. WO 2009/145824 A2 describes a lubricating oil composition comprising polyol ester and polyoxyalkylenealchohol in a range of 0.002% by weight to 2.0% by weight. WO 2013/010851 A1 describes a lubricating oil composition wherein a control constituent has an oxygen/carbon weight ratio in the range of 0.080 to 0.350.

### Citation List

### Patent Literature

PTL 1: WO2013/146805

### Summary of Invention

### Technical Problem

However, a lubricating oil composition used in instruments such as turbines which may be contaminated with water or steam is emulsified by contamination with water or steam, which is a factor causing troubles in instruments.

For this reason, the lubricating oil composition used in such instruments is required to be hardly emulsified and to be easily separated from water even when emulsified, that is, to be excellent in water separability.

In PTL 1, studies have not been conducted on water separability of the lubricating oil composition.

An object of the present invention is to provide a lubricating oil composition excellent in oxidation stability and having a strong effect of preventing sludge precipitation even when used for a long period of time under high temperature environments, and having excellent water separability, wherein the lubricating oil composition is used in turbomachinery, compressors, hydraulic equipments, or machine tools.

### Solution to Problem

The present inventors have found that a lubricating oil composition containing a mixed base oil that contains a combination of a predetermined mineral oil and a synthetic oil containing a polyalkylene glycol (hereinafter also referred to as "PAG") and a polyol ester (hereinafter also referred to as "POE") can solve the above-mentioned problems and have completed the present invention.

That is, the present invention provides the following [1] and [2].
[1] A lubricating oil composition containing a mineral oil (A) and a synthetic oil (B) that contains a polyalkylene glycol (B1) and a polyol ester (B2);
   in which the content of the mineral oil (A) is from 5 to 95% by mass based on the total amount of the lubricating oil composition, and
   which is used in turbomachinery, compressors, hydraulic equipments, or machine tools, as further defined in claim 1.
[2] A method of using a lubricating oil composition, using the lubricating oil composition of the above [1] in turbomachinery, compressors, hydraulic equipments, or machine tools.

### Advantageous Effects of Invention

The lubricating oil composition of the present invention is excellent in oxidation stability, has a strong effect of preventing sludge precipitation and has excellent water separability, even when used for a long period of time under high temperature environments. Consequently, the lubricating oil composition is suitable for use in turbomachinery, compressors, hydraulic equipments, or machine tools.

### Description of Embodiments

In the following description, kinematic viscosity and viscosity index mean values measured and calculated in accordance with JIS K2283:2000.

The content of a phosphorus atom or a metal atom means a value measured in accordance with JPI-5S-38-92.

The content of a nitrogen atom means a value measured in accordance with JIS K2609.

### [Lubricating Oil Composition]

The lubricating oil composition of the present invention is used in turbomachinery, compressors, hydraulic equipments, or machine tools, and contains a mineral oil (A) and a synthetic oil (B) that contains a polyalkylene glycol (PAG) (B1) and a polyol ester (POE) (B2).

The lubricating oil composition of the present invention uses, as a base oil, a mixed base oil containing a synthetic oil that contains PAG and POE, along with a mineral oil (A), and therefore can be excellent in oxidation stability, can have a strong effect of preventing sludge precipitation and can have excellent water separability, even when used for a long period of time under high temperature environments.

Mineral oil is excellent in water separability but is poor in oxidation stability in high-temperature environments and readily forms deterioration materials, and the deterioration materials precipitate as sludge to cause system troubles.

PAG has a property that dissolves deterioration materials to form in high-temperature environments and therefore prevents precipitation of the deterioration materials as sludge, but has a problem in water separability. In addition, since the polarity thereof is too high, PAG is poor in compatibility with an apolar base oil such as mineral oil, and therefore in a mixed base oil of a mineral oil and PAG, the two oils could hardly exhibit a property of compensating for their drawbacks.

On the other hand, POE is poorer than PAG in point of solubility of deterioration materials that form in high-temperature environments, but has a property of being excellent in compatibility with other base oils, and is therefore well compatible with both PAG and mineral oil. However, POE is also problematic in point of water separability.

Consequently, in the present invention, three kinds of base oils, mineral oil, PAG and POE are combined to provide a lubricating oil composition capable of expressing both the characteristic of "mineral oil" excellent in water separability and the characteristic of "PAG" capable of dissolving deterioration materials to form in high-temperature environments, in a well-balanced manner.

In the case where a base oil containing PAG and POE but not containing a mineral oil is used, it still has a problem in point of water separability, and when any other additive is added thereto, the water separability of the resultant base oil tends to further decrease.

On the other hand, in the case where a base oil containing a mineral oil and POE but not containing PAG is used, the base oil is poorer than PAG alone in point of the ability to dissolve deterioration materials to form in high-temperature environments.

Further, in the case where a base oil containing a mineral oil and PAG but not containing POE is used, the compatibility between the mineral oil and PAG is poor, and therefore the characteristic that the mineral oil has and the characteristic that PAG has could be hardly expressed.

In other words, in the present invention, three kinds of base oils, mineral oil, PAG and POE are combined, and therefore, while taking advantages of their own characteristics, it is possible to compensate for the disadvantageous of the individual base oil components by the other constituent base oils.

As a result, the lubricating oil composition of the present invention is excellent in oxidation stability, has a strong effect of preventing sludge precipitation and has excellent water separability, even in use for a long period of time in high-temperature environments.

From the viewpoint of providing such a lubricating oil composition that is excellent in oxidation stability and has a strong effect of preventing sludge precipitation even in use for a long period of time in high-temperature environments, a lubricating oil composition of one embodiment of the present invention preferably further contains an antioxidant (C) containing an amine-based antioxidant (C1).

Also from the viewpoint of improving wear resistance, a lubricating oil composition of one embodiment of the present invention preferably further contains one or more phosphorus compounds (D) selected from a neutral phosphate (D1), an acid phosphate (D2) and an acid phosphate amine salt (D3).

With that, a lubricating oil composition of one embodiment of the present invention may contain any other lubricating oil additives than the components (C) and (D) within a range not detracting from the advantageous effects of the present invention.

In the lubricating oil composition of one embodiment of the present invention, the total content of the components (A) and (B) is, based on the total amount (100% by mass) of the lubricating oil composition, generally 65% by mass or more, preferably 70% by mass or more, more preferably 80% by mass or more, even more preferably 90% by mass or more, further more preferably 95% by mass or more, and is generally 100% by mass or less, preferably 99.9% by mass or less.

In the lubricating oil composition of one embodiment of the present invention, the total content of the components (A), (B), (C) and (D) is, based on the total amount (100% by mass) of the lubricating oil composition, preferably 70 to 100% by mass, more preferably 80 to 100% by mass, even more preferably 90 to 100% by mass, further more preferably 97 to 100% by mass.

The components contained in the lubricating oil composition of one embodiment of the present invention are described below.

### <Mineral Oil (A)>

Examples of the mineral oil (A) for use in the present invention include topped crudes obtained through atmospheric distillation of crude oils such as paraffin-based crude oils, intermediate-based crude oils and naphthene-based crude oils; distillates obtained through reduced-pressure distillation of such topped crudes; mineral oils obtained by purifying the distillates through one or more purification treatments of solvent deasphalting, solvent extraction, hydrocracking, solvent dewaxing, catalytic dewaxing, or hydrorefining; and mineral oil waxes obtained by isomerizing a wax produced from a natural gas through Fischer-Tropsch synthesis (GTL wax (Gas To Liquids WAX)).

One alone or two or more kinds of these mineral oils may be used either singly or as combined.

The mineral oil (A) for use in one embodiment of the present invention is preferably a mineral oil grouped in Group 2 or 3 in the base oil category of API (American Petroleum Institute).

The kinematic viscosity at 40°C of the mineral oil (A) for use in one embodiment of the present invention is preferably 8 to 350 mm²/s, more preferably 10 to 150 mm²/s, even more preferably 12 to 100 mm²/s, further more preferably 15 to 68 mm²/s.

The viscosity index of the mineral oil (A) for use in one embodiment of the present invention is preferably 80 or more, more preferably 90 or more, even more preferably 100 or more.

In the lubricating oil composition of the present invention, the content of the component (A) is, based on the total amount (100% by mass) of the lubricating oil composition, 5 to 95% by mass, preferably 10 to 95% by mass, more preferably 20 to 93% by mass, even more preferably 40 to 92% by mass, further more preferably 60 to 90% by mass.

When the content of the component (A) is less than 5% by mass, the lubricating oil composition is poor in water separability and especially when various additives are added thereto, reduction in water separability of the composition may be greater.

On the other hand, when the content of the component (A) is more than 95% by mass, the content of the components (B1) and (B2) could not be secured sufficiently and, if so, sludge precipitation readily occurs in high-temperature environments and the lubricating oil composition is poor in oxidation stability.

In the lubricating oil of one embodiment of the present invention, the content ratio of the component (A) to the total content of the component (B1) and the component (B2) [(A)/(B 1)+(B2)] is, by mass, from the viewpoint of providing a lubricating oil composition excellent in water separability, preferably 0.05 or more, more preferably 0.10 or more, even more preferably 0.30 or more, further more preferably 0.70 or more, further more preferably 1.50 or more, especially more preferably 3.50 or more, and is, from the viewpoint of providing a lubricating oil composition excellent in oxidation stability and having a strong effect of preventing sludge precipitation even in use for a long period of time in high-temperature environments, preferably 19.0 or less, more preferably 15.0 or less, even more preferably 12.0 or less.

### <Synthetic Oil (B)>

The synthetic oil (B) contained in the lubricating oil composition of the present invention contains a polyalkylene glycol (B1) and a polyol ester (B2).

The synthetic oil (B) for use in one embodiment of the present invention may further contain any other synthetic oil than the components (B1) and (B2) within a range not detracting from the advantageous effects of the present invention.

However, in the lubricating oil composition of one embodiment of the present invention, the total content of the components (B1) and (B2) in the synthetic oil (B) is, based on the total amount (100% by mass) of the synthetic oil (B) contained in the lubricating oil composition, preferably 70 to 100% by mass, more preferably 80 to 100% by mass, even more preferably 90 to 100% by mass, further more preferably 95 to 100% by mass.

In the lubricating oil composition of one embodiment of the present invention, the content ratio of the component (B1) to the component (B2) [(B1)/(B2)] is, by mass, from the viewpoint of providing a lubricating oil composition excellent in oxidation stability and having a strong effect of preventing sludge precipitation even in use for a long period of time in high-temperature environments, preferably 10/90 to 80/20, more preferably 15/85 to 70/30, even more preferably 20/80 to 60/40, further more preferably 25/75 to 55/45.

In the lubricating oil composition of one embodiment of the present invention, the content of the component (B) is, based on the total amount (100% by mass) of the lubricating oil composition, from the viewpoint of providing a a lubricating oil composition excellent in oxidation stability and having a strong effect of preventing sludge precipitation even in use for a long period of time in high-temperature environments, preferably 5% by mass or more, more preferably 6% by mass or more, even more preferably 7% by mass or more, further more preferably 8% by mass or more, and is, from the viewpoint of providing a lubricating oil composition excellent in water separability, preferably 95% by mass or less, more preferably 90% by mass or less, even more preferably 80% by mass or less, further more preferably 60% by mass or less, further more preferably 40% by mass or less, especially more preferably 20% by mass or less.

### [Polyalkylene Glycol (B1)]

Examples of the polyalkylene glycol (B1) include polymers obtained by polymerization or copolymerization of alkylene oxide.

Further, the polyalkylene glycol (B1) may be used alone or in combination of two or more kinds thereof.

A number average molecular weight (Mn) of the polyalkylene glycol (B1) used the present invention is 320 to 1,500 from the viewpoint of improving the viscosity index of the lubricating oil composition.

In this description, the number average molecular weight (Mn) is a value as expressed in terms of standard polystyrene, measured by gel permeation chromatography (GPC), and measurement conditions include conditions described in Examples.

Further, the polyalkylene glycol (B1) used in one embodiment of the present invention is preferably a polyalkylene glycol in which at least one end is sealed with a substituent, from the viewpoint of providing a lubricating oil composition which is further improved in the effect of preventing sludge precipitation.

Examples useful for understanding the invention of the substituent capable of sealing the end of the polyalkylene glycol include a monovalent hydrocarbon group having 1 to 10 carbon atoms, an acyl group having 2 to 10 carbon atoms, or a heterocyclic group having 3 to 10 ring atoms, and preferably, a monovalent hydrocarbon group having 1 to 10 carbon atoms.

Further, examples of specific groups regarding the monovalent hydrocarbon group, acyl group, and heterocyclic group that can be selected as the substituent, and the range of the preferable number of the carbon atoms or ring atoms is the same as defined in R^{B1} and R^{B3} in the following formula (b-1).

In the present invention, the polyalkylene glycol (B1) is a compound represented by the following general formula (b-1), from the viewpoint of providing a lubricating oil composition which is further improved in the effect of preventing sludge precipitation.

R^{B1}-[(OR^{B2})ₐ-OR^{B3}]_{b} (b-1)

In the general formula (b-1), R^{B1} is a hydrogen atoms.

R^{B2} is an alkylene group having 3 to 4 carbon atoms.

R^{B3} is a monovalent hydrocarbon group as defined in claim 1.

b is an integer of 1.

a is a number of 1 or more, and is a value appropriately determined according to the value of the number average molecular weight of the compound represented by the general formula (b-1).

Further, when two or more different kinds of the compound represented by general formula (b-1) are used, a is an average value (a weighted average value), and the average value may be 1 or more.

Further, when there are a plurality of R^{B2} and R^{B3}, R^{B2} and R^{B3} may be the same as or different from each other.

R^{B3} is a monovalent hydrocarbon group selected from the group consisting of a propyl group (a n-propyl group, an isopropyl group), a butyl group (a n-butyl group, an isobutyl group, an s-butyl group, a t-butyl group), a pentyl group, a hexyl group, a cyclopentyl group, a cyclohexyl group, a methylcyclohexyl group, an ethylcyclohexyl group, a propylcyclohexyl group, and a dimethyl cyclohexyl group; a naphthyl group; a benzyl group, a phenylethyl, a methylbenzyl group, a phenylpropyl group, and a phenylbutyl group.

Further, the alkyl group may be either linear or branched.

The number of carbon atoms of the monovalent hydrocarbon group is preferably 1 to 10, more preferably 1 to 6, and still more preferably 1 to 4.

Examples of the alkylene group that can be selected as R^{B2} include an alkylene group having 3 carbon atoms, such as a trimethylene group (-CH₂CH₂CH₂-), a 1-methylethylene group (a propylene group) (-CH(CH₃)CH₂-); and an alkylene group having 4 carbon atoms, such as a tetramethylene group (-CH₂CH₂CH₂CH₂-), a 1-methyltrimethylene group (-CH(CH₃)CH₂CH₂-), a 2-methyltrimethylene group (-CH₂CH(CH₃)CH₂-), a butylene group (-C(CH₃)₂CH₂-), a 1-ethylethylene group (-CH(CH₂CH₃)CH₂-, and a 1,2-dimethylethylene group (-CH(CH₃)-CH(CH₃)-).

Further, when there are a plurality of R^{B2}'s, R^{B2}'s may be the same as each other or may be a combination of two or more kinds of alkylene groups.

Among them, R^{B2} is preferably a 1-methylethylene group (propylene group) (-CH(CH₃)CH₂-).

In the compound represented by the general formula (b-1), the content of the oxypropylene unit (-OCH(CH₃)CH₂-) is preferably 50% by mol to 100% by mol, more preferably 65% by mol to 100% by mol, and still more preferably 80% by mol to 100% by mol, based on the total amount (100% by mol) of the oxyalkylene unit (OR^{B2}) in the structure of the compound.

The kinematic viscosity at 40°C of the component (B1) used in one embodiment of the present invention is preferably 8 mm²/s to 350 mm²/s, more preferably 10 mm²/s to 150 mm²/s, still more preferably 12 mm²/s to 100 mm²/s, and even still more preferably 15 mm²/s to 68 mm²/s.

Further, the viscosity index of the component (B1) used in one embodiment of the present invention is preferably 90 or more, more preferably 100 or more, still more preferably 120 or more, and even still more preferably 140 or more.

In the lubricating oil composition of the present invention, the content of the component (B1) is, based on the total amount (100% by mass) of the lubricating oil composition, 1.0 to 70% by mass, more preferably 1.2 to 50% by mass, even more preferably 1.4 to 30% by mass, further more preferably 1.5 to 20% by mass, further more preferably 1.7 to 12% by mass, and especially more preferably 1.9 to 6% by mass.

### [Polyol Ester (B2)]

Examples of the polyol ester (B2) include a hindered ester of a hindered polyol, which has one or more quaternary carbon atoms in the molecule wherein at least one of the quaternary carbon atoms has 1 to 4 methylol groups bonded thereto, with an aliphatic monocarboxylic acid.

The polyol ester (B2) may be used alone or in combination of two or more kinds thereof.

Further, the polyol ester (B2) is generally a complete ester in which all the hydroxy groups of the polyol are esterified, but may include a partial ester in which some of the hydroxy groups remain unesterified, as long as the effects of the present invention are not impaired.

The hindered polyol is preferably a compound represented by the following general formula (b-2).

In the general formula (b-2), R^{B11} and R^{B12} are each independently a monovalent hydrocarbon group having 1 to 6 carbon atoms or a methylol group (-CH₂OH).

n represents an integer of 0 to 4, preferably 0 to 2, more preferably 0 or 1, and still more preferably 0. When n = 0, it is a single bond and provides a compound represented by the following general formula (b-2').

In the general formula (b-2'), R^{B11} and R^{B12} each independently represent a monovalent hydrocarbon group having 1 to 6 carbon atoms or a methylol group (-CH₂OH).

Examples of the monovalent hydrocarbon group having 1 to 6 carbon atoms which can be selected as R^{B11} and R^{B12} include alkyl groups having 1 to 6 carbon atoms (a methyl group, an ethyl group, a propyl group, a butyl group, a pentyl group, a hexyl group), a cyclopentyl group, a cyclohexyl group, and a phenyl group.

Further, the alkyl group may be either linear or branched.

Among them, the monovalent hydrocarbon group having 1 to 6 carbon atoms which can be selected as R^{B11} and R^{B12} is preferably an alkyl group having 1 to 6 carbon atoms, and more preferably an alkyl group having 1 to 3 carbon atoms.

Examples of the compound represented by the following general formula (b-2) include a hindered polyol such as a dialkylpropanediol (wherein the alkyl group has 1 to 6 carbon atoms), a trimethylolalkane (wherein the alkane has 2 to 7 carbon atoms), and a pentaerythritol, and a dehydrated condensate thereof, and more specifically, neopentyl glycol, 2-ethyl-2-methyl-1,3-propanediol, 2,2-diethyl 1,3-propanediol, trimethylolethane, trimethylolpropane, trimethylolbutane, trimethylolpentane, trimethylolhexane, trimethylolheptane, pentaerythritol, 2,2,6,6-tetramethyl-4-oxa-1,7-heptanediol, 2,2,6,6,10,10-hexamethyl-4,8-dioxa-1,11-undecadiol, 2,2,6,6,10,10,14,14-octamethyl-4,8,12-trioxa-1,15-pentadecadiol, 2,6-di(hydroxymethyl)-2,6-dimethyl-4-oxa-1,7-heptanediol, 2,6,10-tri(hydroxymethyl)-2,6,10-trimethyl-4,8-dioxa-1,11-undecadiol, 2,6,10,14-tetra(hydroxymethyl)-2,6,10,14-tetramethyl-4,8,12-trioxa-1,15-pentadecadiol, di(pentaerythritol), tri(pentaerythritol), tetra(pentaerythritol), and penta(pentaerythritol).

Among them, trimethylolpropane, neopentyl glycol, pentaerythritol, and bimolecular or trimolecular dehydrated condensates thereof are preferred, and trimethylolpropane, neopentyl glycol, and pentaerythritol are more preferred, and trimethylolpropane is still more preferred.

The aliphatic monocarboxylic acid includes a saturated aliphatic monocarboxylic acid having 5 to 22 carbon atoms.

The acyl group of the saturated aliphatic monocarboxylic acid may be either linear or branched.

Examples of the saturated aliphatic monocarboxylic acid include a linear saturated monocarboxylic acid such as valeric acid, caproic acid, enanthic acid, caprylic acid, pelargonic acid, capric acid, undecanoic acid, lauric acid, tridecanoic acid, myristic acid, pentadecanoic acid, palmitic acid, heptadecanoic acid, stearic acid, nonadecanoic acid, arachic acid, and behenic acid; and a branched saturated monocarboxylic acid such as isomyristic acid, isopalmitic acid, isostearic acid, 2,2-dimethylpropanoic acid, 2,2-dimethylbutanoic acid, 2,2-dimethylpentanoic acid, 2,2-dimethyloctanoic acid, 2-ethyl-2,3,3-trimethylbutanoic acid, 2,2,3,4-tetramethylpentanoic acid, 2,5,5-trimethyl-2-t-butylhexanoic acid, 2,3,3-trimethyl-2-ethylbutanoic acid, 2,3-dimethyl-2-isopropylbutanoic acid, 2-ethylhexanoic acid, and 3,5,5-trimethylhexanoic acid.

In esterification, these aliphatic monocarboxylic acids may be used alone or in combination of two or more kinds thereof.

The number of carbon atoms of the saturated aliphatic monocarboxylic acid is preferably 5 to 18, more preferably 6 to 14, and still more preferably 8 to 10.

The kinematic viscosity at 40°C of the polyol ester (B2) used in one embodiment of the present invention is preferably 8 mm²/s to 350 mm²/s, more preferably 10 mm²/s to 150 mm²/s, still more preferably 11 mm²/s to 100 mm²/s, and even still more preferably 12 mm²/s to 68 mm²/s.

Further, the viscosity index of the polyol ester (B2) used in one embodiment of the present invention is preferably 90 or more, more preferably 100 or more, still more preferably 110 or more, and even still more preferably 120 or more.

The number average molecular weight (Mn) of the polyol ester (B2) used in one embodiment of the present invention is preferably 100 to 8,000, more preferably 200 to 4,000, still more preferably 300 to 2,000, and even still more preferably 400 to 1,000.

In the lubricating oil composition of the present invention, the content of the component (B2) is, based on the total amount (100% by mass) of the lubricating oil composition, 2.0 to 90% by mass, more preferably 2.5 to 70% by mass, even more preferably 3.0 to 55% by mass, further more preferably 3.5 to 40% by mass, further more preferably 4.0 to 30% by mass, and especially more preferably 4.5 to 15% by mass.

### [Synthetic Oil other than Components (B1) and (B2)]

The synthetic oil (B) for use in one embodiment of the present invention may further contain any other synthetic oil than the components (B1) and (B2) within a range not detracting from the advantageous effects of the present invention.

Examples of the other synthetic oil include poly-α-olefins such as α-olefin homopolymers or α-olefin copolymers (for example, α-olefin copolymers having 8 to 14 carbon atoms such as ethylene-α-olefin copolymers); isoparaffin; various esters other than the component (B2), such as dibasic acid esters (for example, ditridecyl glutarate), aromatic acid esters (for example, 2-ethylhexyl trimellitate, 2-ethylhexyl pyromellitate), and phosphate esters; various ethers other than the component (B 1), such as polyphenyl ethers; alkylbenzenes; and alkylnaphthalenes.

One alone or two or more kinds of these synthetic oils may be used either singly or as combined.

### <Antioxidant (C)>

The lubricating oil composition of one embodiment of the present invention preferably contains an antioxidant (C) containing an amine-based antioxidant (C1), from the viewpoint of providing a lubricating oil composition which is excellent in oxidation stability, suppresses generation of deterioration products, and is further improved in the effect of preventing sludge precipitation.

The antioxidant (C) used in one embodiment of the present invention may further contain any other antioxidant than the amine-based antioxidant (C1) together with the amine-based antioxidant (C1).

In the lubricating oil composition of one embodiment of the present invention, the content of the component (C 1) in the component (C) is, based on the total amount (100% by mass) of the component (C), preferably 30 to 100% by mass, more preferably 50 to 100% by mass, even more preferably 60 to 100% by mass, and further more preferably 70 to 100% by mass, from the viewpoint of providing a lubricating oil composition which suppresses generation of deterioration products, is further improved in the effect of preventing sludge precipitation, and has excellent oxidation stability.

In the lubricating oil composition of one embodiment of the present invention, the content of the component (C) is preferably 0.01 to 10% by mass, more preferably 0.05 to 7% by mass, and still more preferably 0.1 to 5% by mass, based on the total amount (100% by mass) of the lubricating oil composition, from the viewpoint of providing a lubricating oil composition which suppresses generation of deterioration products, is further improved in the effect of preventing sludge precipitation, and has excellent oxidation stability.

### [Amine-based Antioxidant (C1)]

The amine-based antioxidant (C1) may be an amine-based compound having antioxidant performance, and includes naphthylamine (C11) and diphenylamine (C12).

The amine-based antioxidant (C1) may be used alone or in combination of two or more kinds thereof.

Further, in one embodiment of the present invention, both naphthylamine (C11) and diphenylamine (C12) are preferably included.

In the lubricating oil composition of one embodiment of the present invention, the content ratio [(C11)/(C12)] of the naphthylamine (C11) and the diphenylamine (C12) is preferably 10/90 to 90/10, more preferably 15/85 to 85/15, still more preferably 20/80 to 80/20, and even still more preferably 25/75 to 75/25 by a mass ratio.

Examples of the naphthylamine (C11) include phenyl-α-naphthylamine, phenyl-β-naphthylamine, alkylphenyl-α-naphthylamine, and alkylphenyl-β-naphthylamine, and preferably, alkylphenyl-α-naphthylamine and alkylphenyl-β-naphthylamine.

The number of carbon atoms of the alkyl group in the alkylphenyl-α-naphthylamine and the alkylphenyl-β-naphthylamine is preferably 1 to 30, but is, from the viewpoint of improving solubility with the mineral oil (A) and the synthetic oil (B), and more improving the effect of preventing sludge precipitation, more preferably 1 to 20, even more preferably 4 to 16, and still more preferably 6 to 14.

The diphenylamine (C12) is preferably a compound represented by the following general formula (c-1) and more preferably a compound represented by the following general formula (c-2).

In the general formulae (c-1) and (c-2), R^{x} and R^{y} are each independently an alkyl group having 1 to 30 carbon atoms, or an alkyl group having 1 to 30 carbon atoms substituted with an aryl group having 6 to 18 ring atoms.

The alkyl group may be either a linear alkyl group or a branched alkyl group.

In general formula (c-1), z1 and z2 are each independently an integer of 0 to 5, preferably 0 or 1, and more preferably 1. Further, when there are a plurality of R^{x} and R^{y}, R^{x} and R^{y} may be the same as or different from each other.

Further, the number of carbon atoms of the alkyl group which can be selected as R^{x} and R^{y} is 1 to 30, preferably 1 to 20, and more preferably 1 to 10.

Examples of the aryl group that can be substituted for the alkyl group include a phenyl group, a naphthyl group, and a biphenyl group, and preferably, a phenyl group.

Examples of the alkyl group in the alkylphenyl-naphthylamine and the alkyl group in the diphenylamine include a methyl group, an ethyl group, a propyl group, a butyl group, a pentyl group, a hexyl group, a heptyl group, an octyl group, a nonyl group, a decyl group, an undecyl group, a dodecyl group, a hexadecyl group, an octadecyl group, a nonadecyl group, an eicosyl group, and a tetracosyl group.

In the lubricating oil composition of one embodiment of the present invention, the content of the amine-based antioxidant (C1) in terms of nitrogen atom is preferably 50 to 3000 ppm by mass, more preferably 100 to 2000 ppm by mass, still more preferably 120 to 1500 ppm by mass, even still more preferably 150 to 1000 ppm by mass, based on the total amount (100% by mass) of the lubricating oil composition, from the viewpoint of providing a lubricating oil composition which suppresses generation of deterioration products, is further improved in the effect of preventing sludge precipitation, and has excellent oxidation stability.

### [Antioxidant other than amine-based antioxidant (C 1)]

The antioxidant (C) may also contain an antioxidant other than the above amine-based antioxidant (C1). As such an antioxidant, a phenol-based antioxidant is preferred.

Examples of the phenol-based antioxidant include monocyclic phenol compounds such as 2,6-di-t-butyl-4-methylphenol, 2,6-di-t-butyl-4-ethylphenol, 2,4,6-tri-t-butylphenol, 2,6-di-t-butyl-4-hydroxymethylphenol, 2,6-di-t-butylphenol, 2,4-dimethyl-6-t-butylphenol, 2,6-di-t-butyl-4-(N,N-dimethylaminomethyl)phenol, 2,6-di-t-amyl-4-methylphenol, and n-octadecyl-3-(3,5-di-t-butyl-4-hydroxyphenyl)propionate; and polycyclic phenol compounds such as 4,4'-methylenebis(2,6-di-t-butylphenol), 4,4'-isopropylidenebis(2,6-di-t-butylphenol), 2,2'-methylenebis(4-methyl-6-t-butylphenol), 4,4'-bis(2,6-di-t-butylphenol), 4,4'-bis(2-methyl-6-t-butylphenol), 2,2'-methylenebis(4-ethyl-6-t-butylphenol), and 4,4'-butylidenebis(3-methyl-6-t-butylphenol).

In the lubricating oil composition of one embodiment of the present invention, the content of the phenol-based antioxidant relative to 100 parts by mass of the amine-based antioxidant (C1) is preferably 0 part by mass to 100 parts by mass, more preferably 0 part by mass to 60 parts by mass, and still more preferably 0 part by mass to 40 parts by mass.

### <Phosphorus Compound (D)>

The lubricating oil composition of one embodiment of the present invention preferably further contains one or more phosphorus compounds (D) selected from a neutral phosphate (D1), an acid phosphate (D2), an acid phosphate amine salt (D3) and a sulfur-phosphorus compound (D4), from the viewpoint of improving wear resistance.

From the viewpoint of further improving rust-preventing performance, the component (D) preferably contains one or more selected from the component (D1) and the component (D3). Also from the viewpoint of satisfying both oxidation stability and wear resistance even in a relatively small amount, the component (D) preferably contains one or more selected from the component (D3) and the component (D4).

In the lubricating oil composition of one embodiment of the present invention, the content of the component (D) in terms of phosphorus atom is, based on the total amount (100% by mass) of the lubricating oil composition, preferably 10 to 1600 ppm by mass, more preferably 20 to 1200 ppm by mass, even more preferably 50 to 1000 ppm by mass, further more preferably 100 to 800 ppm by mass, especially more preferably 150 to 600 ppm by mass. In the case where one or more selected from the component (D3) and the component (D4) are used, the content thereof in terms of phosphorus atom may be, based on the total amount (100% by mass) of the lubricating oil composition, preferably 10 to 50 ppm by mass, more preferably 10 to 30 ppm by mass.

In the lubricating oil composition of one embodiment of the present invention, the content of the component (D) is, based on the total amount (100% by mass) of the lubricating oil composition, preferably 0.01 to 2.0% by mass, more preferably 0.02 to 1.5% by mass, even more preferably 0.05 to 1.0% by mass, further more preferably 0.10 to 0.70% by mass. When one or more selected from the component (D3) and the component (D4) are used, the content of the component (D) may be, based on the total amount (100% by mass) of the lubricating oil composition, preferably 0.01 to 1.0 ppm by mass, more preferably 0.01 to 0.2 ppm by mass, even more preferably 0.01 to 0.05 ppm by mass.

### [Neutral Phosphate (D1)]

The neutral phosphate (D1) is preferably a compound (D11) represented by the following general formula (d1-1).

In the general formula (d1-1), R^{D1} to R^{D3} are each independently an alkyl group having 1 to 18 (preferably 3 to 18) carbon atoms, or an aryl group having 6 to 18 ring carbon atoms and substituted with an alkyl group having 1 to 18 (preferably 3 to 12) carbon atoms.

Examples of the alkyl group having 1 to 18 carbon atoms which can be selected as R^{D1} to R^{D3} include a methyl group, an ethyl group, a propyl group (a n-propyl group, an isopropyl group), a butyl group (a n-butyl group, an s-butyl, a t-butyl group, an isobutyl group), a pentyl group, a hexyl group, a 2-ethyl hexyl group, a heptyl group, an octyl group, a nonyl group, a decyl group, an undecyl group, a dodecyl group, a tridecyl group, a tetradecyl group, a pentadecyl group, a hexadecyl group, a heptadecyl group, and an octadecyl group.

These alkyl group may be either a linear alkyl group or a branched alkyl group.

Examples of the aryl group having 6 to 18 ring carbon atoms include a phenyl group, a naphthyl group, an anthryl group, a phenanthryl group, a biphenyl group, a terphenyl group, and a phenylnaphthyl group, and preferably, a phenyl group.

The "aryl group substituted with an alkyl group having 1 to 18 carbon atoms" which can be selected as R^{D1} to R^{D3} includes a group in which at least one of hydrogen atoms bonded to the ring carbon atoms of the aryl group is substituted with the alkyl group having 1 to 18 carbon atoms.

The compound (D11) is more preferably a compound (D12) represented by the following general formula (d1-2).

In the general formula (d1-2), R^{D11} to R^{D13} are each independently an alkyl group having 1 to 18 carbon atoms. The alkyl group may be the same as the alkyl group which can be selected as R^{D11} to R^{D13}.

The number of carbon atoms of the alkyl group which can be selected as R¹¹ to R¹³ is 1 to 18 but is, from the viewpoint of providing a lubricating oil composition having improved rust-preventing performance, preferably 3 to 12, more preferably 3 to 8, even more preferably 3 to 6, further more preferably 3.

p1 to p3 are each independently an integer of 1 to 5, preferably an integer of 1 to 2, and more preferably 1.

### [Acid Phosphate (D2)]

The acid phosphate (D2) is preferably one or more selected from a compound represented by the following general formula (d2-1) and a compound represented by the following general formula (d2-2).

In the general formulae (d2-1) and (d2-2), R^{a} and R^{b} are each independently an alkyl group having 1 to 12 carbon atoms. The alkyl group may be the same as the alkyl group having 1 to 12 carbon atoms among the alkyl group which can be selected as R^{D1} to R^{D3} as mentioned above.

The number of carbon atoms of the alkyl group which can be selected as R^{a} and R^{b} is preferably 3 to 10, more preferably 6 to 10, and still more preferably 8 to 10.

R^{a} and R^{b} in the general formula (d2-1) may be the same as or different from each other.

### [Acid Phosphate Amine Salt (D3)]

The acid phosphate amine salt (D3) is preferably one or more selected from an amine salt of a compound represented by the above-mentioned general formula (d2-1) and an amine salt of a compound represented by the above-mentioned general formula (d2-2).

The amine to form the amine salt is preferably a compound represented by the following general formula (d3). One alone or two or more kinds of the amines may be used either singly or as combined.

(R^{c})_{q}-N-(H)_{3-q} (d3)

In the general formula (d3), q represents an integer of 1 to 3.

R^{C} is each independently an alkyl group having 6 to 18 carbon atoms, an alkenyl group having 6 to 18 carbon atoms, an aryl group having 6 to 18 ring carbon atoms, an arylalkyl group having 7 to 18 carbon atoms, or a hydroxyalkyl group having 6 to 18 carbon atoms, and preferably, an alkyl group having 6 to 18 carbon atoms.

When there are a plurality of R^{C}s, R^{C}s may be the same as or different from each other.

Examples of the alkyl group which can be selected as R^{C} include a hexyl group, a heptyl group, an octyl group, a 2-ethylhexyl group, a nonyl group, a decyl group, an undecyl group, a dodecyl group, a tridecyl group, a tetradecyl group, a hexadecyl group, and an octadecyl group.

The alkyl group may be either a linear alkyl group or a branched alkyl group.

The number of carbon atoms of the alkyl group which can be selected as R^{C} is 6 to 18, preferably 7 to 16, more preferably 8 to 15, and still more preferably 10 to 13.

Examples of the alkenyl group which can be selected as R^{C} include a hexenyl group, a heptenyl group, an octenyl group, a nonenyl group, a decenyl group, an undecenyl group, a dodecenyl group, a tridecenyl group, a tetradecenyl group, a hexadecenyl group, and an octadecenyl group.

The alkenyl group may be either a linear alkenyl group or a branched alkenyl group.

The number of carbon atoms of the alkenyl group which can be selected as R^{C} is 6 to 18, preferably 7 to 16, more preferably 8 to 15, and still more preferably 10 to 13.

Examples of the aryl group which can be selected as R^{C} include a phenyl group, a naphthyl group, an anthryl group, a phenanthryl group, a biphenyl group, a terphenyl group, and a phenylnaphthyl group.

The number of carbon atoms of the aryl group which can be selected as R^{C} is 6 to 18, preferably 6 to 16, and more preferably 6 to 14.

The arylalkyl group which can be selected as R^{C} includes a group in which a hydrogen atom of the alkyl group is substituted with the aryl group, and specifically, a phenylmethyl group, and a phenylethyl group.

The number of carbon atoms of the arylalkyl group which can be selected as R^{C} is 7 to 18, preferably 7 to 16, and more preferably 8 to 14.

The hydroxyalkyl group which can be selected as R^{C} includes a group in which a hydrogen atom of the alkyl group is substituted with a hydroxy group, and specifically, a hydroxyhexyl group, a hydroxyoctyl group, a hydroxydodecyl group, and a hydroxytridecyl group.

The number of carbon atoms of the hydroxyalkyl group which can be selected as R^{C} is 6 to 18, preferably 7 to 16, more preferably 8 to 15, and still more preferably 10 to 13.

### [Sulfur-Phosphorus Compound (D4)]

The sulfur-phosphorus compound (D4) includes monothiophosphates, dithiophosphates, trithiophosphates, monothiophosphate amine salts, dithiophosphate amine salts, monothiophosphites, dithiophosphites, and trithiophosphites, and among these, dithiophosphates are preferred.

From the viewpoint of bettering wear resistance, dithiophosphates having a carboxy group or an ester residue at the terminal are preferred among dithiophosphates. Having a carboxy group or an ester group at the terminal, the sulfur-phosphorus compound (D4) can have high polarity, and therefore also in this embodiment using the above-mentioned specific ester-based synthetic base oil (A) as a base oil, the sulfur-phosphorus compound of the type can readily exhibit a function as an extreme pressure agent.

Specific examples of the dithiophosphate having a carboxy group or an ester residue at the terminal include compounds represented by the following general formula (d4).

In the formula (d4), R^{d} represents a linear or branched alkylene group having 1 to 8 carbon atoms, R^{e} and R^{f} each independently represent a hydrocarbon group having 1 to 20 carbon atoms. R^{g} represents a hydrogen atom or a hydrocarbon group having 1 to 10 carbon atoms.

In the formula (d4), R^{d} is from the viewpoint of bettering solubility in base oil, preferably a linear or branched alkylene group having 1 to 8 carbon atoms, more preferably a linear or branched alkylene group having 2 to 4 carbon atoms, even more preferably an alkylene group having 2 carbon atoms or a branched alkylene group having 3 to 4 carbon atoms. Specifically, -CH₂CH₂-, -CH₂CH(CH₃)-, -CH₂CH(CH₂CH₃)-, -CH₂CH(CH₃)CH₂-, and -CH₂CH(CH₂CH₂CH₃)- are preferred; -CH₂CH₂-, -CH₂CH(CH₃)-, and -CH₂CH(CH₃)CH₂- are more preferred; and -CH₂CH₂-, and -CH₂CH(CH₃)- are even more preferred.

R^{e} and R^{f} each are, from the viewpoint of bettering extreme pressure performance and bettering solubility in base oil, preferably a linear or branched alkyl group having 1 to 8 carbon atoms, more preferably a linear or branched alkyl group having 3 to 6 carbon atoms. Specifically, they are preferably selected from groups of propyl, isopropyl, butyl, isobutyl, t-butyl, pentyl, isopentyl, hexyl, 2-ethylbutyl, 1-methylpentyl, 1,3-dimethylbutyl and 2-ethylhexyl, and among these, isopropyl, isobutyl and t-butyl are more preferred.

R^{g} is, from the viewpoint of bettering extreme pressure performance and solubility in base oil, preferably a hydrogen atom, or a linear or branched alkyl group having 1 to 4 carbon atoms. Specifically, a hydrogen atom and groups of methyl, ethyl, propyl, isopropyl, butyl, isobutyl and t-butyl group are preferred, and among these, a hydrogen atom, a methyl group and an ethyl group are more preferred.

### <Other Additives for Lubricating Oil>

The lubricating oil composition of one embodiment of the present invention may contain any other additive for lubricating oil than the above-mentioned components (B) to (D) within a range not detracting from the advantageous effects of the present invention.

Examples of such additives for lubricating oil include a rust inhibitor, a detergent dispersant, a viscosity index improver, an anti-foaming agent, a friction modifier, and a metal deactivator.

One alone or two or more kinds of these additives for lubricating oil may be used either singly or as combined.

In the case where such additives for lubricating oil are added, the content of each additive for lubricating oil may be appropriately controlled depending on the kind of the additive within a range not detracting from the advantageous effects of the present invention, but is, based on the total amount (100% by mass) of the lubricating oil composition, generally 0.001 to 10% by mass, preferably 0.005 to 5% by mass, more preferably 0.01 to 2% by mass.

A lubricating oil composition prepared by blending an alkenylsuccinate in a base oil of PAG or POE suffers from worsening of water separability.

However, the lubricating oil composition of the present invention contains a base oil (A) that is well compatible with an alkenylsuccinate and therefore can effectively exhibit rust-preventing performance that the alkenylsuccinate has. In addition, even though an alkenylsuccinate is blended therein, the lubricating oil composition can still have good water separability.

In the lubricating oil composition of one embodiment of the present invention, the content of the alkenylsuccinate is, based on the total amount (100% by mass) of the lubricating oil composition, preferably 0.001 to 5.0% by mass, more preferably 0.005 to 2.0% by mass, even more preferably 0.01 to 1.0% by mass, further more preferably 0.02 to 0.50% by mass.

Preferably, the lubricating oil composition of one embodiment of the present invention does not substantially contain a metal atom-containing compound from the viewpoint of preventing sludge precipitation to occur in use for a long period of time in high-temperature environments.

Here, the metal atom in the "metal atom-containing compound" includes an alkali metal atom, an alkaline earth metal atom and a transition metal atom.

In this description, "does not substantially contain a metal atom-containing compound" is a definition to deny an embodiment of incorporating a metal atom-containing compound with a predetermined object but is not a definition to deny even a case of containing a metal atom-containing compound as an impurity.

However, the content of a metal atom-containing compound contained as an impurity is preferably as small as possible.

In the lubricating oil composition of one embodiment of the present invention, the content of a metal atom is, from the viewpoint of preventing sludge precipitation to occur in use for a long period of time in high-temperature environments, based on the total amount (100% by mass) of the lubricating oil composition, preferably less than 100 ppm by mass, more preferably less than 50 ppm by mass, even more preferably less than 10 ppm by mass, further more preferably less than 5 ppm by mass.

In this description, the content of a metal atom means a value measured according to JPI-5S-38-92.

### [Physical Properties of Lubricating Oil Composition]

The kinematic viscosity at 40°C of the lubricating oil composition of one embodiment of the present invention is preferably 5 to 300 mm²/s, more preferably 10 to 200 mm²/s, even more preferably 15 to 100 mm²/s.

The viscosity index of the lubricating oil composition of one embodiment of the present invention is preferably 90 or more, more preferably 100 or more, even more preferably 105 or more, further more preferably 110 or more.

When the lubricating oil composition of one embodiment of the present invention is tested according to the oxidation stability test (Dry-TOST method) of ASTM D7873, the amount of sludge precipitated in 960 hours after the start of the test in an environment of 120°C is preferably 1.0 mg/100 ml or less, more preferably 0.7 mg/100 ml or less, even more preferably 0.5 mg/100 ml or less.

The amount of the precipitated sludge is a value measured in accordance with ASTM D7873 using a membrane filter having an average pore diameter of 1.0 µm.

When the lubricating oil composition of one embodiment of the present invention is tested under environment of 120°C according to the oxidation stability test (Dry-TOST method) of ASTM D7873, the RPVOT residual ratio in 960 hours after the start of the test is preferably 65% or more, more preferably 70% or more, even more preferably 72% or more.

RPVOT residual ratio is a value calculated according to the following expression. [RPVOT residual ratio] (%) = [RPVOT time of sample after test]/[RPVOT time of sample before test] × 100

When the lubricating oil composition of one embodiment of the present invention is tested in a water separability test at a temperature of 54°C according to JIS K2520, the demulsibility degree that indicates a time to be taken for an emulsion layer to reach 3 mL is preferably 15 minutes or less, more preferably 10 minutes or less, even more preferably 5 minutes or less.

The traction coefficient of the lubricating oil composition of one embodiment of the present invention, as measured under the measurement conditions shown in the section of Examples given hereinunder, is preferably 0.020 or less, more preferably 0.018 or less.

### [Use of Lubricating Oil Composition, and Lubrication Method]

The lubricating oil composition of the present invention is used in turbomachinery, compressors (excepting refrigerators), hydraulic equipments, or machine tools.

Specifically, the lubricating oil composition of one embodiment of the present invention is favorably used as a lubricating oil (pump oil, turbine oil) for turbomachinery for use for lubrication of turbomachinery such as pumps, vacuum pumps, blowers, turbocompressors, steam turbines, atomic force turbines, gas turbines, and turbines for hydraulic power generation; a bearing oil, a gear oil or a control system operating oil for lubrication for compressors such as rotary compressor and reciprocating compressors; a hydraulic actuation oil for use for hydraulic machines; and a lubricating oil for machine tools for use for hydraulic units of machine tools.

Namely, the present application also provides a use method of the following [1],
[1] A method of using a lubricating oil composition, using a lubricating oil composition containing a mineral oil (A) and a synthetic oil (B) that contains a polyalkylene glycol (B1) and a polyol ester (B2), in which the content of the mineral oil (A) is 5 to 95% by mass, in turbomachinery, compressors, hydraulic equipments, or machine tools.

Specific constitutions of the lubricating oil composition of the present invention, as well as specific exemplifications of turbomachinery, compressors, hydraulic equipments, and machine tools are as described above.

### Examples

The present invention is described more specifically with reference to Examples, but the present invention is not limited to these Examples.

### [Measurement methods of various physical property values]

(1) Kinematic viscosity, Viscosity index
   Measured and calculated in accordance with JIS K2283:2000.
(2) Number average molecular weight (Mn)
   Mn was measured in terms of standard polystyrene according to gel permeation chromatography (GPC) under the following measurement conditions.
   (Measurement conditions)
   Gel permeation chromatography apparatus: "1260 type HPLC" manufactured by Agilent Co.
   Standard sample: polystyrene
   Column: One in which two of "Shodex LF404" were successively connected to each other
   Column temperature: 35°C
   Developing solvent: Chloroform
   Flow rate: 0.3 mL/min
(3) Contents of phosphorus and metal atoms
   Measured in accordance with JPI-5S-38-92.
(4) Contents of nitrogen atom
   Measured in accordance with JIS K2609.

### Examples 1 to 7 and Comparative Examples 1 to 5

The mineral oil, synthetic oil, amine-based antioxidant, phosphorus compound and other additives shown below were blended at the blending ratio shown in Table 1 and, and fully mixed to prepare lubricating oil compositions (I) to (VII) and (i) to (v), respectively.

The details of the respective components used in the preparation of the lubricating oil compositions are as mentioned below.

### (Mineral oil)

"150N Mineral Oil": mineral oil grouped in Group 2 of the API base oil category. Kinematic viscosity at 40°C = 30.6 mm²/s, viscosity index = 104. (Synthetic oil)

"PAG": Polypropylene glycol of which one end is sealed with butyl ether which is represented by H-(OCH(CH₃)CH₂)ₐ-OC₄H₉ (in the general formula (b-1), R^{B1} is a hydrogen atom, R^{B2} is a propylene group, R^{B3} is a n-butyl group, and b is 1). Kinematic viscosity at 40°C = 37.2 mm²/s, viscosity index = 173, Mn = 800.

"POE": Trimethylolpropane triester (complete ester of trimethylolpropane and carboxylic acid having 8 to 10 carbon atoms). Kinematic viscosity at 40°C = 19.6 mm²/s, viscosity index = 138.

### (Amine-based antioxidant)

"Naphthylamine": P-octylphenyl-α-naphthylamine. Nitrogen atom content = 4.2% by mass.

"Diphenylamine": Bis(p-octylphenyl)amine, a compound represented by the general formula (c-2) where R^{x} and R^{y} are octyl group. Nitrogen atom content = 3.6% by mass.

### (Phosphorus compound)

"Neutral phosphate ester": Tris(p-isopropylphenyl)phosphate, in the general formula (d1-2), p1 to p3 are 1, and R^{D11} to R^{D13} are isopropyl groups, wherein the isopropyl group is bonded to the para-position. Phosphorus atom content = 6.8% by mass.

"Acid phosphate amine": Amine salt of a mixture of a compound represented by the general formula (d2-1) and a compound represented by the general formula (d2-2), and a compound represented by the general formula (d3). (In the general formula (d2-1) and the general formula (d2-2), R^{a} and R^{b} each are an alkyl group having 8 or 10 carbon atoms, in the general formula (d3), R^{c} is an alkyl group having 12 carbon atoms, q is 1 or 2.) Phosphorus atom content = 4.8% by mass.

Thiophosphate 1: 3-Diisobutoxyphosphinothioylsulfanyl-2-methylpropanoic acid. Phosphorus atom content = 9.3% by mass.

Thiophosphate 2: Ethyl-3-[{bis(1-methylethoxy)phosphinothioyl}thio]propionate. Phosphorus atom content = 9.9% by mass.

### (Other additives)

"Rust inhibitor": Alkenylsuccinate half ester.

"Anti-foaming agent": Silicone-based anti-foaming agent, acryl-based anti-foaming agent.

With respect to each of the prepared lubricating oil compositions, various physical property values shown in Tables 1 and 2 were measured according to the above methods, and various properties of the lubricating oil compositions were evaluated by conducting the following tests. The results are shown in Tables 1 and 2.

### (1) Oxidation stability test (Dry-TOST)

The amount of sludge precipitated and the RPVOT residual ratio in 960 hours after initiation of the test under environment of 120°C was measured in accordance with the oxidation stability test (Dry-TOST) of ASTM D7873.

The amount of the precipitated sludge was measured in accordance with ASTM D7873 using a membrane filter having an average pore diameter of 1.0 µm (provided by Millipore Corporation).

The RPVOT residual ratio was calculated according to the following expression. [RPVOT residual ratio] (%) = [RPVOT time of sample after test]/[RPVOT time of sample before test] × 100

### (2) Water separability test

A water separability test was conducted at a temperature of 54°C in accordance with JIS K2520 to measure the time (demulsibility unit: min) taken for an emulsion layer to reach 3 mL.

### (3) Measurement of traction coefficient

Using an EHD oil film measuring device (available from PCS Instruments Ltd.), a traction coefficient was measured under the following measurement conditions.
Disc: diameter 46 mm, SAE AISI52100 steel
Ball: diameter 19 mm, SAE AISI52100 steel
Load: 20 N
Rolling speed: 2.0 m/s
Oil temperature: 60°C
Slip ratio: 10%

### (4) Wear resistance test

Using an FZG gear tester and according to ISO 14635-1, a load was stepwise increased as prescribed, and a stage under a load to have generated scouring was evaluated. A higher stage of load indicates more excellent scouring resistance.

The lubricating oil compositions prepared in Examples 1 to 7 were excellent in oxidation stability and had a strong effect of preventing sludge precipitation, and and had excellent water separability. In addition, these have a low traction coefficient and showed an effect of improving wear resistance.

On the other hand, the lubricating oil composition prepared in Comparative Example 1 was poor in oxidation stability, and as compared with those in Examples, this caused much sludge precipitation and had a low RPVOT residual ratio. In addition, this is insufficient in point of wear resistance.

The lubricating oil compositions prepared in Comparative Examples 2, 3, 4 and 5 had good oxidation stability and wear resistance, but were poor in water separability, and among these, the composition of Comparative Example 4 was especially poor in oxidation stability, and caused relatively much sludge precipitation.

## Claims

1. A lubricating oil composition comprising a mineral oil (A) and a synthetic oil (B) that comprises a polyalkylene glycol (B1) and a polyol ester (B2);
in which the content of the mineral oil (A) is from 5 to 95% by mass based on the total amount of the lubricating oil composition,
wherein the content of the component (B1) is 1.0 to 70% by mass based on the total amount of the lubricating oil composition,
wherein the content of the component (B2) is 2.0 to 90% by mass based on the total amount of the lubricating oil composition,
which is used in turbomachinery, compressors, hydraulic equipments, or machine tools, and
wherein the polyalkylene glycol (B1) is a compound represented by the following general formula (b-1), and
R^{B1}-[(OR^{B2})ₐ-OR^{B3}]_{b} (b-1)
wherein in the general formula (b-1),
a is a number of 1 or more,
b is an integer of 1,
R^{B1} is a hydrogen atom,
R^{B2} is an alkylene group having 3 or 4 carbon atoms,
R^{B3} is a monovalent hydrocarbon group selected from the group consisting of a propyl group, a butyl group, a pentyl group, a hexyl group, a cyclopentyl group, a cyclohexyl group, a methylcyclohexyl group, an ethylcyclohexyl group, a propylcyclohexyl group, and a dimethyl cyclohexyl group, a naphthyl group, a benzyl group, a phenylethyl, a methylbenzyl group, a phenylpropyl group, and a phenylbutyl group, and
wherein a number average molecular weight (Mn) of the polyalkylene glycol (B1) is 320 to 1,500, as measured by gel permeation chromatography.

2. The lubricating oil composition according to claim 1, wherein the content ratio of the component (B1) to the component (B2) [(B1)/(B2)] is, by mass, from 10/90 to 80/20.

3. The lubricating oil composition according to claim 1 or 2, wherein the content ratio of the component (A) to the total content of the component (B1) and the component (B2) [(A)/((B1)+(B2))] is, by mass, from 0.05 to 19.0.

4. The lubricating oil composition according to any one of claims 1 to 3, further comprising an antioxidant (C) that comprises an amine-type antioxidant (C 1).

5. The lubricating oil composition according to claim 4, wherein the nitrogen atom-equivalent content of the component (C1) is, based on the total amount of the lubricating oil composition, from 50 to 3,000 ppm by mass.

6. The lubricating oil composition according to any one of claims 1 to 5, further comprising one or more phosphorus compounds (D) selected from a neutral phosphate (D1), an acid phosphate (D2), an acid phosphate amine salt (D3) and a sulfur-phosphorus compound (D4).

7. The lubricating oil composition according to claim 6, wherein the phosphorus atom-equivalent content of the component (D) is, based on the total amount of the lubricating oil composition, from 10 to 1,600 ppm by mass.

8. The lubricating oil composition according to any one of claims 1 to 7, wherein the metal atom content is, based on the total amount of the lubricating oil composition, less than 100 ppm by mass.

9. The lubricating oil composition according to any one of claims 1 to 8, wherein, when the lubricating oil composition is tested in a water separability test at a temperature of 54°C according to JIS K2520, the demulsibility degree that indicates a time to be taken for an emulsion layer to reach 3 mL is 15 minutes or less.

10. A method of using a lubricating oil composition, using the lubricating oil composition of any one of claims 1 to 9 in turbomachinery, compressors, hydraulic equipments, or machine tools.

## Patentansprüche

1. Schmierölzusammensetzung, umfassend ein Mineralöl (A) und ein synthetisches Öl (B), das ein Polyalkylenglycol (B1) und einen Polyolester (B2) umfasst;
wobei der Gehalt des Mineralöls (A) 5 bis 95 Massen-%, bezogen auf die Gesamtmenge der Schmierölzusammensetzung, beträgt,
wobei der Gehalt der Komponente (B1) 1,0 bis 70 Massen-%, bezogen auf die Gesamtmenge der Schmierölzusammensetzung, beträgt,
wobei der Gehalt der Komponente (B2) 2,0 bis 90 Massen-%, bezogen auf die Gesamtmenge der Schmierölzusammensetzung, beträgt,
die in Turbomaschinen, Kompressoren, hydraulischen Geräten oder Werkzeugmaschinen verwendet wird, und wobei das Polyalkylenglycol (B1) eine Verbindung, dargestellt durch die folgende allgemeine Formel (b-1) ist, und
R^{B1}-[(OR^{B2})ₐ-OR^{B3}]_{b} (b-1)
wobei in der allgemeinen Formel (b-1)
a eine Zahl von 1 oder mehr ist,
b eine ganze Zahl von 1 ist,
R^{B1} ein Wasserstoffatom ist,
R^{B2} eine Alkylengruppe mit 3 oder 4 Kohlenstoffatomen ist,
R^{B3} eine monovalente Kohlenwasserstoffgruppe ist, die aus der Gruppe ausgewählt ist, die aus einer Propylgruppe, einer Butylgruppe, einer Pentylgruppe, einer Hexylgruppe, einer Cyclopentylgruppe, einer Cyclohexylgruppe, einer Methylcyclohexylgruppe, einer Ethylcyclohexylgruppe, einer Propylcyclohexylgruppe und einer Dimethylcyclohexylgruppe, einer Naphthylgruppe, einer Benzylgruppe, einer Phenylethylgruppe, einer Methylbenzylgruppe, einer Phenylpropylgruppe und einer Phenylbutylgruppe besteht, und
wobei das zahlenmittlere Molekulargewicht (Mn) des Polyalkylenglycols (B1) 320 bis 1500, gemessen durch Gelpermeationschromatographie, beträgt.

2. Schmierölzusammensetzung gemäß Anspruch 1, wobei das Gehaltsmassenverhältnis von der Komponente (B1) zu der Komponente (B2) [(B1)/(B2)] 10/90 bis 80/20 beträgt.

3. Schmierölzusammensetzung gemäß Anspruch 1 oder 2, wobei das Gehaltsmassenverhältnis von der Komponente (A) zu dem Gesamtgehalt der Komponente (B1) und der Komponente (B2) [(A)/((B1)+(B2))] 0,05 bis 19,0 beträgt.

4. Schmierölzusammensetzung gemäß einem der Ansprüche 1 bis 3, ferner umfassend ein Antioxidationsmittel (C), das ein Antioxidationsmittel vom Amintyp (C1) umfasst.

5. Schmierölzusammensetzung gemäß Anspruch 4, wobei der Gehalt des Stickstoffatomäquivalents der Komponente (C1), 50 bis 3000 Massen-ppm, bezogen auf die Gesamtmenge der Schmierölzusammensetzung, beträgt.

6. Schmierölzusammensetzung gemäß einem der Ansprüche 1 bis 5, ferner umfassend eine oder mehrere Phosphorverbindungen (D), die aus einem neutralen Phosphat (D1), einem sauren Phosphat (D2), einem sauren Phosphataminsalz (D3) und einer Schwefel-PhosphorVerbindung (D4) ausgewählt sind.

7. Schmierölzusammensetzung gemäß Anspruch 6, wobei der Gehalt des Phosphoratomäquivalents der Komponente (D) 10 bis 1600 Massen-ppm, bezogen auf die Gesamtmenge der Schmierölzusammensetzung, beträgt.

8. Schmierölzusammensetzung gemäß einem der Ansprüche 1 bis 7, wobei der Metallatomgehalt weniger als 100 Massen-ppm, bezogen auf die Gesamtmenge der Schmierölzusammensetzung, beträgt.

9. Schmierölzusammensetzung gemäß einem der Ansprüche 1 bis 8, wobei, wenn die Schmierölzusammensetzung in einem Wasserabtrenntest bei einer Temperatur von 54°C gemäß JIS K2520 getestet wird, der Demulgierbarkeitsgrad, der eine Zeit angibt, die eine Emulsionsschicht benötigt, um 3 ml zu erreichen, 15 Minuten oder weniger beträgt.

10. Verfahren zur Verwendung einer Schmierölzusammensetzung, bei dem die Schmierölzusammensetzung gemäß einem der Ansprüche 1 bis 9 in Turbomaschinen, Kompressoren, hydraulischen Geräten oder Werkzeugmaschinen verwendet wird.

## Revendications

1. Composition d'huile lubrifiante comprenant une huile minérale (A) et une huile synthétique (B) qui comprend un polyalkylène glycol (B1) et un ester de polyol (B2) ;
dans laquelle la teneur en huile minérale (A) est de 5 à 95 % en masse par rapport à la quantité totale de la composition d'huile lubrifiante,
dans laquelle la teneur du composant (B1) est de 1,0 à 70 % en masse par rapport à la quantité totale de la composition d'huile lubrifiante,
dans laquelle la teneur du composant (B2) est comprise entre 2,0 et 90 % en masse par rapport à la quantité totale de la composition d'huile lubrifiante,
qui est utilisée dans des turbomachines, des compresseurs, des équipements hydrauliques, ou des machines-outils, et
dans laquelle le polyalkylène glycol (B1) est un composé représenté par la formule générale suivante (b-1), et
R^{B1}-[(OR^{B2})_{B}-OR^{B3}]_{b} (b-1)
dans laquelle, dans la formule générale (b-1),
a est un nombre de 1 ou plus,
b est un nombre entier de 1,
R^{B1} est un atome d'hydrogène,
R^{B2} est un groupe alkylène présentant 3 ou 4 atomes de carbone,
R^{B3} est un groupe hydrocarboné monovalent choisi dans le groupe constitué par un groupe propyle, un groupe butyle, un groupe pentyle, un groupe hexyle, un groupe cyclopentyle, un groupe cyclohexyle, un groupe méthylcyclohexyle, un groupe éthylcyclohexyle, un groupe propylcyclohexyle, et un groupe diméthylcyclohexyle, un groupe naphtyle, un groupe benzyle, un groupe phényléthyle, un groupe méthylbenzyle, un groupe phénylpropyle, et un groupe phénylbutyle, et
dans laquelle le poids moléculaire moyen en nombre (Mn) du polyalkylène glycol (B1) est compris entre 320 et 1 500, tel que mesuré par chromatographie par perméation de gel.

2. Composition d'huile lubrifiante selon la revendication 1, dans laquelle le rapport de teneur entre le composant (B1) et le composant (B2) [(B1)/(B2)] est, en masse, de 10/90 à 80/20.

3. Composition d'huile lubrifiante selon la revendication 1 ou la revendication 2, dans laquelle le rapport de teneur entre le composant (A) et la teneur totale du composant (B1) et du composant (B2) [(A)/((B1)+(B2))] est, en masse, compris entre 0,05 et 19,0.

4. Composition d'huile lubrifiante selon l'une quelconque des revendications 1 à 3, comprenant en outre un antioxydant (C) qui comprend un antioxydant de type amine (C1).

5. Composition d'huile lubrifiante selon la revendication 4, dans laquelle la teneur en équivalent d'atome d'azote du composant (C1) est, par rapport à la quantité totale de la composition d'huile lubrifiante, de 50 à 3 000 ppm en masse.

6. Composition d'huile lubrifiante selon l'une quelconque des revendications 1 à 5, comprenant en outre un ou plusieurs composés phosphorés (D) choisis parmi un phosphate neutre (D1), un phosphate acide (D2), un sel d'amine de phosphate acide (D3) et un composé soufre-phosphore (D4).

7. Composition d'huile lubrifiante selon la revendication 6, dans laquelle la teneur en équivalent d'atome de phosphore du composant (D) est, par rapport à la quantité totale de la composition d'huile lubrifiante, de 10 à 1 600 ppm en masse.

8. Composition d'huile lubrifiante selon l'une quelconque des revendications 1 à 7, dans laquelle la teneur en atomes métalliques est, par rapport à la quantité totale de la composition d'huile lubrifiante, inférieure à 100 ppm en masse.

9. Composition d'huile lubrifiante selon l'une quelconque des revendications 1 à 8, dans laquelle, lorsque la composition d'huile lubrifiante est soumise à un test de séparabilité de l'eau à une température de 54 °C conformément à la norme JIS K2520, le degré de désémulsibilité qui indique le temps nécessaire pour qu'une couche d'émulsion atteigne 3 ml est de 15 minutes ou moins.

10. Procédé d'utilisation d'une composition d'huile lubrifiante, utilisant la composition d'huile lubrifiante selon l'une quelconque des revendications 1 à 9 dans des turbomachines, des compresseurs, des équipements hydrauliques, ou des machines-outils.
